

3,068,100  
N-ACYLHOMOCYSTEINE THIOLACTONE STABILIZERS FOR PHOTOGRAPHIC SILVER HALIDE EMULSIONS

Fritz Dersch, Binghamton, N.Y., assignor to General Aniline &amp; Film Corporation, a corporation of Delaware

No Drawing. Filed Nov. 14, 1960, Ser. No. 68,653  
20 Claims. (Cl. 96—66)

This invention relates to photographic materials and to methods of preparing them. More particularly, this invention relates to light-sensitive silver halide emulsions containing as a stabilizing and antifogging agent an N-acyl DL-homocysteine thiolactone.

It is well known in the photographic art that light-sensitive emulsions such as gelatino-silver halide emulsions have a tendency to fog. Fog is usually caused by a prolonger ripening of the emulsion, by prolonged storage especially at elevated temperatures and humidity and by prolonged development. To overcome this undesirable property, it has been the practice in this art to add certain chemical compounds to the emulsions to increase their stability and to reduce their tendency to fog. However, the stabilizing and antifogging compounds heretofore used in this art have the disadvantage that upon addition to the emulsion they cause a loss of speed and/or contrast of the emulsion.

It is, accordingly, an object of this invention to produce a light-sensitive emulsion which is fast, stable, has a reduced tendency to fog and has good contrast.

A further object of this invention resides in a light-sensitive emulsion which contains a compound which stabilizes the emulsion against fogging and at the same time does not materially reduce the speed and/or the contrast of the emulsion.

I have discovered that N-acyl DL-homocysteine thiolactones when added to a light-sensitive silver halide emulsion, stabilize and inhibit the fogging of the emulsion. The N-acyl DL-homocysteine thiolactones, the use of which is contemplated herein, may be represented by the following formula:



wherein R is a low alkyl radical; for example, methyl, ethyl, propyl or isopropyl.

The following specific compounds are examples of compounds belonging to the class of compounds having the general formula given above which I have found suitable for use as stabilizing and antifogging agents.



N-acetyl DL-homocysteine thiolactone



N-propionyl DL-homocysteine thiolactone



N-butyryl DL-homocysteine thiolactone

These compounds are prepared by treating DL-homocysteine thiolactone hydroiodide prepared according to the method described in J. Biol. Chem., volume 106, page 451 (1934), with silver acetate and reacting the free base with a suitable anhydride such as acetic anhydride, propionic anhydride or butyric anhydride.

15. The antifogging agents of my invention may be added to the emulsion at any stage during its process of production. Thus, they may be added as a "ripening final" or as a "coating final." When added as a "ripening final," they are added during the ripening or sensitivity increasing stage of the emulsion-making process. Such addition may be made before, during or after the addition of the soluble silver salt to the soluble halide in the presence of a suitable colloid such as gelatin, polyvinyl alcohol, solubilized casein or albumin which may be used as the carrier material. When added as a coating final, the antifogging agent of my invention is added to the emulsion just prior to coating it on a suitable support such as glass, paper or film at a time when the emulsion has nearly attained its maximum sensitivity. In some instances, it is advantageous to apply the antifogging and stabilizing compounds of my invention in a separate layer such as an under coating layer or in an anti-abrasion gelatin surface. Sometimes it is desirable to incorporate the compounds in one or all processing baths; for instance, in the developer solution or in the pre-bath which is used prior to development.

When used as a "ripening final," the antifoggants of my invention are preferably added to the emulsion in an amount ranging from 0.1 milligram to 60 milligrams per 0.6 mol of silver halide; and when used as a "coating final," they are preferably added in an amount ranging from 10 milligrams to 300 milligrams per 0.6 mol of silver halide. The optimum amount to be added depends primarily on the type of emulsion and should be determined individually in each case.

The stabilizers and antifoggants of my invention may also be used in combination with known antifoggants and stabilizers; the antifoggants of my invention can also be used in combination with sensitizers such as sulfur, metal and reduction sensitizers as well as with speed-increasing agents and accelerators such as the reaction products of long-chain alcohols and ethylene oxide (see United States Patent 1,907,578) and their derivatives.

The novel antifoggants of my invention may be used with various types of photographic emulsions such as non-sensitized orthochromatic, panchromatic and X-ray emulsions, paper emulsions and color emulsions.

60. The following specific examples are given as an illustration of the manner in which the antifoggants of my invention can be used. It is to be understood, however, that these examples are given by way of illustration and not by way of limitation.

## PREPARATION

65. A mixture of 12.25 grams of DL-homocysteine thiolactone hydroiodide and 8.35 grams of silver acetate dispersed in 500 milliliters of glacial acetic acid was stirred for 30 minutes at room temperature. The silver iodide which was formed in this reaction was removed by filtration. Ten milliliters of freshly distilled acetic anhydride was added to the filtrate and the mixture allowed to stand for 2 hours. The acetic acid was distilled off in vacuum,

and the residue dried over sodium hydroxide in a vacuum desiccator. The residue was recrystallized from toluene and yielded a product having a melting point of 110° C.

*Example I*

A silver halide emulsion in gelatin containing 2 percent silver iodide and 98 percent silver bromide was prepared in a conventional manner and brought up to its maximum light sensitivity. It was then readied for coating by adding finals such as sensitizing dyes and hardening agents. A 0.1 percent solution of N-acetyl DL-homocysteine thiolactone prepared as described above was added in varying amounts to samples of the emulsion as an antifogging and stabilizer. Each emulsion sample contained about 0.6 mol of silver halide. The so prepared emulsion samples were coated on a suitable cellulose ester base and dried. Samples of these film coatings were then exposed in a Type IIB Sensitometer and developed in a developer of the following composition:

|                                     | Grams |
|-------------------------------------|-------|
| Metol (p-methylaminophenol sulfate) | 1.5   |
| Sodium sulfite (anhydrous)          | 45.0  |
| Sodium bisulfite                    | 1.0   |
| Hydroquinone                        | 3.0   |
| Sodium carbonate (monohydrate)      | 6.0   |
| Potassium bromide                   | 0.8   |
| Water to make 1.0 liter.            |       |

The developed samples were short-stopped, fixed and washed and dried. The results obtained were as follows:

| Quantity of compound used | Relative speed | Fog at 12 min. development | Oven fog at 6 min. development |
|---------------------------|----------------|----------------------------|--------------------------------|
| 0                         | 100            | .25                        | .20                            |
| 15 mg.                    | 100            | .15                        | .10                            |
| 30 mg.                    | 100            | .14                        | .10                            |
| 50 mg.                    | 95             | .13                        | .10                            |

*Example II*

The procedure followed was identical to Example I except that in place of N-acetyl DL-homocysteine thiolactone the compound used was N-propionyl DL-homocysteine thiolactone prepared in an analogous manner except that propionic anhydride was used in place of acetic anhydride.

The results obtained were substantially identical with those of Example I.

*Example III*

The procedure followed was identical to Example I but in place of N-acetyl DL-homocysteine thiolactone was used the compound N-butyryl DL-homocysteine thiolactone which had been prepared by using butyric anhydride in place of acetic anhydride.

The results obtained were very similar to those of Example I.

*Example IV*

Several examples of a conventional film were exposed in a Type IIB Sensitometer and then divided into two groups. One group of samples was developed for twelve minutes at 68° F. in a standard metol hydroquinone developer as described in Example I. The second group of samples was developed for the same length of time and at the same temperature as the first group in a metol hydroquinone developer which had been prepared by adding to the developer described in Example I 10 mgs. of N-acetyl DL-homocysteine thiolactone per liter of developer. It was found that both sets of samples had the same relative speed of 100. However, the samples developed in the control developer showed a fog of .30 whereas the strips which had been developed in the presence of the antifogging showed a fog of 0.20.

*Example V*

One kilo of a silver halide emulsion in gelatin containing 4 percent silver iodide and 96 percent silver bromide was coated on film base in a manner known to the art. After the coating was performed, an aqueous gelatin solution containing 20 grams of gelatin per liter and 1.2 grams of the N-acetyl DL-homocysteine thiolactone of Example I was coated thereon as an antiabrasion layer. After 10 drying, film samples were exposed and processed as described in Example I. The samples described exhibited a relative speed of 100 with a fog of .12 as compared with a type coating of the same emulsion having an antiabrasion layer similar to that described above but lacking the antifogging additive and having a speed of 100 and a fog of .20.

Modifications of the invention will occur to persons skilled in the art. I do not intend to be limited in the patent granted except as necessitated by the appended 20 claims.

I claim:

I. A light-sensitive silver halide emulsion containing in a stabilizing amount an antifogging compound having the following general chemical formula:



wherein R is a lower alkyl group of from 1 to 3 carbon atoms.

2. A light-sensitive silver halide emulsion as recited in claim 1 wherein the antifogging and stabilizing compound is N-acetyl DL-homocysteine thiolactone.

3. A light-sensitive silver halide emulsion as recited in claim 1 wherein the antifogging and stabilizing compound is N-propionyl DL-cysteine thiolactone.

4. A light-sensitive silver halide emulsion as recited in claim 1 wherein the antifogging and stabilizing compound is present in the emulsion in the ratio of 0.1 to 300 milligrams per 0.6 mol of silver halide.

5. A light-sensitive silver halide emulsion as recited in claim 1 containing a sensitizing dye.

6. A light-sensitive silver halide emulsion as recited in claim 1 containing the reaction product of a long chain alcohol and an ethylene oxide as an accelerator.

7. A light-sensitive photographic element comprising a base and a coating of gelatin silver halide emulsion thereon said emulsion containing as an antifogging and stabilizing agent a compound having the following general formula:



60 65 wherein R is an alkyl group of from 1 to 3 carbon atoms.

8. A light-sensitive photographic element according to claim 7 wherein said compound is N-acetyl DL-homocysteine thiolactone.

9. A light-sensitive photographic element according to claim 7 wherein said compound is N-propionyl DL-cysteine thiolactone.

10. A light-sensitive structure comprising a base, a layer of a light-sensitive silver halide emulsion thereon and a separate layer adjacent to and in contiguous contact with said first-mentioned layer containing as an anti-

fogging and stabilizing agent a compound selected from the group having the following general structure:



wherein R is a member selected from the group consisting of methyl, ethyl and propyl.

11. A light-sensitive structure as defined by claim 10 wherein said compound is N-acetyl DL-homocysteine thiolactone.

12. A process of forming a light-sensitive photographic element having a reduced tendency to fog which comprises forming an emulsion, ripening said emulsion, coating said emulsion on a base and adding to said emulsion just prior to the coating thereof on the base a compound having the following general formula:



wherein R is a member selected from the group consisting of methyl, ethyl and propyl.

13. A process according to claim 12 wherein said compound is N-acetyl DL-homocysteine thiolactone.

14. A process of forming a photographic emulsion having a reduced tendency to fog which comprises forming the emulsion, ripening the emulsion and during said ripening adding thereto a compound having the following general formula:



wherein R is an alkyl group of from 1 to 3 carbon atoms.

15. A process according to claim 14 wherein said compound is N-acetyl DL-homocysteine thiolactone.

16. The process of minimizing and preventing fog on light-sensitive silver halide materials comprising a base having a light-sensitive silver halide emulsion thereon which comprises exposing the emulsion and developing the exposed emulsion in the presence of an antifogging amount of a compound having the following general formula:



10

15

wherein R represents a member selected from the group consisting of methyl, ethyl and propyl radicals.

17. A process according to claim 16 wherein said antifogging agent is N-acetyl DL-homocysteine thiolactone.

18. A process according to claim 16 wherein said antifogging agent is N-propionyl DL-homocysteine thiolactone.

19. A photographic developer solution comprising an organic developing agent, an alkali, an alkali metal sulfite, an alkali metal bromide and as an antifogging agent, in an antifogging amount, a compound having the following general formula:



30

35 wherein R represents an alkyl group having one to three carbon atoms.

20. A photograph developer solution according to claim 19 wherein said compound is N-acetyl DL-homocysteine thiolactone.

#### References Cited in the file of this patent

#### UNITED STATES PATENTS

- |    |           |                     |               |
|----|-----------|---------------------|---------------|
| 45 | 2,824,001 | Allen et al. -----  | Feb. 18, 1958 |
|    | 2,870,015 | Allen et al. -----  | Jan. 20, 1959 |
|    | 2,939,789 | Dersch et al. ----- | June 7, 1960  |

#### OTHER REFERENCES

- Glafkides: Photographic Chemistry, vol. I, Fountain  
50 Press, London, 1958, pages 374-75.

UNITED STATES PATENT OFFICE  
CERTIFICATE OF CORRECTION

Patent No. 3,068,100

December 11, 1962

Fritz Dersch

It is hereby certified that error appears in the above numbered patent requiring correction and that the said Letters Patent should read as corrected below.

Column 1, line 19, for "prolonger" read -- prolonged --;  
column 2, line 53, for "1,907,578" read -- 1,970,578 --.

Signed and sealed this 3rd day of September 1963.

(SEAL)

Attest:

ERNEST W. SWIDER

Attesting Officer

DAVID L. LADD

Commissioner of Patents